

June 28, 1932.

A. JOFFÉ

1,864,828

ELECTRICAL CONDENSER AND THE LIKE

Filed May 15, 1926



Abraham Joffé Inventor  
By his Attorney  
Edward M. Evans

## UNITED STATES PATENT OFFICE

ABRAHAM JOFFÉ, OF LENINGRAD, RUSSIA, ASSIGNOR TO INDUSTRIAL RESEARCH COMPANY, OF CAMBRIDGE, MASSACHUSETTS, A CORPORATION OF MASSACHUSETTS

## ELECTRICAL CONDENSER AND THE LIKE

Application filed May 15, 1926. Serial No. 109,914.

My present invention relates to capacities, such as condensers, variable and fixed, and the like, and aims to devise devices of the general character specified which are simple in construction, easy and convenient to fabricate and to assemble, and which are characterized by their simple construction, their accuracy and reliability in use, and their resistance to rupture even when highly charged.

10 In the accompanying specification I shall describe, and in the annexed drawing more or less diagrammatically illustrate, an illustrative embodiment of the present invention. It is, however, to be clearly understood that 15 my invention is not limited to the specific form thereof herein shown and described for purposes of illustration only.

Referring to the drawing, wherein I have illustrated the aforesaid illustrative embodiment of the present invention:

Fig. 1 of the drawing shows, more or less diagrammatically, in side elevation, a simple type of capacity or condenser constructed in accordance with the principles of the present 25 invention;

Fig. 2 is a longitudinal sectional view of the device shown in Fig. 1 of the drawing; and

Figs. 3, 4, 5, 6, 7 and 8 are diagrammatic 30 views illustrating current distributions with different arrangements of devices.

Referring now to the aforesaid illustrative embodiment of the present invention, and more particularly to the drawing illustrating 35 the same, 10 and 11 indicate layers or films of conductive material, such as layers or films of aluminum which may be of any desired thickness. These conductive plates or films perform the usual function in the condenser or 40 capacity of serving as the terminal plates to which the poles of the source of high-tension or other current may be connected to charge the condenser or capacity.

Interposed between the conductive plates 45 or films 10 and 11 is a layer or film preferably of a non-crystalline polarizable material of a dielectric, semi-conductive or similar character. This layer or film of polarizable dielectric or like material has been generally 50 designated by reference character 20.

The material 20 is not an ordinary dielectric, insulation or like material, but is rather a non-crystalline material capable of being polarized so as to serve as a storer or accumulator of a charge of electric current having a polarity the magnitude and character of which depends upon the charge impressed upon the positive plate or terminal, here designated by reference character 10. In a co-pending application of mine filed October 28, 55 1925, Serial No. 65,262, and entitled "Utilizing the polarization of dielectric substances traversed by electric currents", I have set forth the basic principles of the property of the class or type of non-crystalline dielectric substances capable of being polarized and capable, for this reason, of being adapted for the purposes of the present invention. The present application is a continuation in part of the earlier filed application just referred to. As set forth in such earlier filed co-pending application, I have previously discovered, as described by me in the article published together with Prof. W. C. Rontgen (Analener Physik, IV, volume 72, page 472) that 60 65 dielectric crystals, that is, crystals of dielectric substances, are polarized upon passing through the same a current at a potential of about or exceeding ten thousand volts. Under such conditions, the electromotive force 70 of the polarization approximates the applied potential.

My investigations have shown that this polarization apparently takes place only in a thin layer of stratum bordering upon the 75 crystal at the surface of the cathode. Moreover, it comprises a condition of ionization. In contradistinction to the ordinary molecular stress extending uniformly through a dielectric irrespective of its thickness, this polarization is therefore a surface or 80 85 90 95 100 ionic polarization. Apparently, the thickness of the material of which the dielectric crystal is made does not have any appreciable influence on the polarization. However, in many instances additional thickness (in addition to the thickness of the polarized layer) is not only useless but objectionable, as for example in high frequency circuits. Consequently an important feature of the invention consists in

confining the thickness of the dielectric to a dimension comparable to the thickness of the aforesaid polarization.

I have discovered, as a result of further extensive researches in this and related fields, that other dielectric substances, of a non-crystalline character, and even semi-conductors, have yielded the wholly unexpected result of becoming similarly polarized upon passing therethrough a current of about or exceeding one or two thousand volts, this unexpected result being obtained when the consistency of such non-crystalline dielectric substances and semi-conductors is tough or sufficiently strong or solid.

For example, I have discovered that satisfactory polarization effects may, under such conditions, be obtained with such substances as calcium carbonate, aluminum phosphate, aluminum oxide, cement, linseed-oil varnish, etc.

While for an insulation for high-tension transmission lines and the like I prefer that the non-crystalline polarizable material shall comprise a linseed oil varnish, made as set forth on later in this specification, and characterized by a relatively low specific capacity and a relatively high specific conductivity, such material may, however, also be used for the purposes of the present invention in the construction of a capacity or condenser made in accordance with the principles of the present invention. Likewise, while for the purpose of an accumulator or storer of high-tension current made in accordance with the principles of my earlier filed copending application referred to above, I prefer to use a non-crystalline inorganic substance like precipitated calcium carbonate or this same substance in the form of the material known as "mother of pearl", characterized by a relatively high specific capacity and a relatively high specific conductivity, I may use this material also for the purposes of the present invention in the construction of a capacity or condenser made in accordance with the principles of the present invention.

I prefer, however, for the specific purposes of the present invention, to use a material characterized by a relatively high specific capacity and a relatively low specific conductivity, such as the material known as boron trioxide. This material is remarkably well suited for use in capacities or condensers made in accordance with the principles of the present invention.

In the case of a linseed oil varnish, for example, while a layer 0.01 mm. in thickness, for an average variety of such varnish, may be ruptured by the sudden application of an electric tension of one thousand volts, if the electric tension is gradually built up over a substantial period of time, as from about one-half to about one second, more or less, such a layer will stand an electric tension of

ten thousand or even fifteen thousand volts before being ruptured.

As an example of such a linseed oil varnish, I may mention a linseed oil varnish made up of linseed oil, containing from about 1 to about 3 per cent. its weight of a suitable drier or oxidizer, dried at an elevated temperature, as from about 100 to about 200° centigrade. For example, where the drying takes place at about 180° centigrade, should be continued for from about two to about three hours.

In order to serve the purposes of the present invention most successfully, it is desirable, even necessary, that the layer or film of the linseed oil varnish be of substantially uniform or even thickness. For this purpose, I prefer that the drying take place on a layer of mercury or other suitable heavy liquid on which the varnish may float during the drying operation, the varnish being preferably dissolved for this purpose in a suitable solvent, such as nitrobenzol.

Such a layer of linseed oil varnish, mother of pearl, or boron trioxide, preferably the latter, will be found to have a capacity for Faradic current up to five thousand, ten thousand, or even fifteen thousand, volts for a thickness of the material of an order of about 0.01 mm. Furthermore, if the voltage is applied gradually and over an appreciable period of time, as from about one-half to about one second, this thin layer of non-crystalline polarizable material in accordance with the principles of the present invention will not be ruptured by such voltages, whereas if the voltage were suddenly applied it might be ruptured by a voltage as low as one thousand volts.

The action of the charge is difficult to ascertain, but it would appear as if the material is polarized or "ionized", thus causing the material to receive an appreciable charge under high tension and adapting it, therefore, for a condenser or capacity characterized by its remarkable capacity, its great strength, its accuracy, and its resistance to rupture.

As already stated, the outer conducting plates 10 and 11 may consist of aluminum or other suitable metallic or other conductive substance. Furthermore, in place of the materials already mentioned as being suitable for use as non-crystalline polarizable substances for the purposes of the present invention, certain organic materials, such as colloidal calcium compounds, or certain inorganic materials, generally of a colloidal character, such as gum or resins, may be employed for the purpose of the present invention.

In concluding the description of the aforesaid illustrative embodiment of the present invention, it may be desirable to indicate the following methods which are suitable for the manufacture of thin dielectric layers suitable for embodiment in the various high-tension polarization devices described above:

- (1) The material may be applied as a coating of tough or colloidal material, after which it may be dried or heated to form a compact, tough layer.
- (2) Alternate layers of "non-conductive", such as semi-conductive or dielectric material, and of metallic layers, may be obtained by sublimation at reduced pressures or in a suitable gas which reacts with the sublimated material and forms the layer of the desired dielectric or semi-conductive substance.
- (3) The desired layer of dielectric or semi-conductive substance may be formed by electrolysis using a further chemical or electrochemical reaction, if necessary, to complete the formation of the desired dielectric or semi-conductive substance.
- (4) The desired dielectric or semi-conductive substance may be formed by cathodic or mechanical dispersion, which latter is also termed the "spraying" or "spouting" method.
- (5) The desired layer of dielectric or semi-conductive substance may be formed by separation from a solution or from a colloidal solution.
- (6) Finally other methods by which thin layers of any suitable material are produced, particularly such mechanical methods as rolling, pressing or the like, may be used for producing the desired dielectric or semi-conductive layers.
- The results of the present invention are numerous and of great practical importance. By means of the polarizable dielectric or like substances of the present invention, especially in non-crystalline condition, such as the linseed oil varnish, "mother of pearl", and boron trioxide described above, and the arrangement of such material in one or more layers together with one or more intervening or surrounding, or intervening and surrounding, layers of metal or other suitable conducting materials, the alternate members of which may be connected to one pole and the remaining members of which may be connected to the other pole of a source of high-tension or other current, it is possible in a simple and highly efficient manner to construct a condenser or capacity, either variable or fixed, which embodies one or more layers of one or more of the various non-crystalline dielectric or like substances of the present invention. The resulting capacities or condensers are characterized by their simplicity in construction, their dependability, their remarkably high capacity and their resistance to rupture.
- Other advantages and superiorities of the capacities and condensers of the present invention will be readily apparent to those skilled in the art to which the present invention relates.
- Referring now to Figs. 3 to 8 inclusive, Fig. 3 shows the distribution of the charge where the wire carries positive electricity, Fig. 4 showing the distribution of the charge where the wire carries negative electricity, Figs. 5 and 6 illustrating the gradients for these respective types of transmission. Figs. 7 and 8 show the gradients for these two types of transmission where the dielectric or semi-conductive substance consists of borax, boron trioxide or borax glass where the polarization produces charges of both signs.
- What I claim as my invention is:
1. A capacitor comprising a plurality of electrically conductive elements and a layer of semi-conductive polarizable material comprising boron trioxide interposed between each pair of said electrically conductive elements of which a layer of a thickness of an order of about 0.01 mm. has a resistance to rupture up to about a voltage of an order of about ten thousand volts under graduated load.
  2. A capacitor comprising a plurality of electrically conductive elements and a layer of semi-conductive non-crystalline polarizable material comprising boron trioxide interposed between each pair of said electrically conductive elements.
  3. A capacitor comprising a plurality of electrically conductive elements and interposed polarizable material comprising boron trioxide.
  4. A capacitor comprising a plurality of electrically conductive elements and a layer of semi-conductive non-crystalline polarizable material comprising boron trioxide interposed between each pair of said electrically conductive elements of which a layer of a thickness of an order of about 0.01 mm. has a resistance to rupture up to about a voltage of an order of about ten thousand volts under graduated load.
  5. A capacitor comprising a plurality of electrically conductive elements and interposed polarizable material comprising boron trioxide of which a layer of a thickness of an order of about 0.01 mm. has a resistance to rupture up to about a voltage of an order of about ten thousand volts under graduated load.
  6. A capacitor comprising a plurality of electrically conductive elements and a layer of semi-conductive polarizable material comprising boron trioxide interposed between each pair of said electrically conductive elements.
  7. The method of producing dielectric capacitor material which comprises subjecting a thin layer of semi-conductive polarizable material of a thickness of an order of about .01 mm., to a gradually increasing voltage up to the order of about one thousand volts.
  8. The method of producing dielectric capacitor material which comprises subjecting a thin layer of semi-conductive polarizable

material to a voltage and gradually increasing the value of said voltage from zero up to a potential gradient of about 1,000,000 volts per centimeter, the thickness of said 5 layer being considerably less than 1 mm.

9. A capacitor including a thin layer of semi-conductive polarizable material of a thickness of an order of about .01 mm. said material having a thin polarized layer 10 formed upon one surface thereof.

10. A capacitor comprising a thin layer of semi-conductive polarizable material, said layer being polarized upon one surface thereof, the insulating strength of said layer being 15 concentrated in said polarized layer so that a voltage which would produce breakdown across an unpolarized layer of the same thickness is insufficient to cause breakdown.

11. The method of producing dielectric capacitor material which comprises subjecting 20 a thin layer of semi-conductive, polarizable material of a thickness of the order of .01 mm. during a period not less than the order of a half a second to a gradually increasing 25 voltage up to the order of about 1000 volts, the said upper limit not being attained until the end of said period.

12. The method of producing dielectric capacitor material which comprises subjecting 30 a sheet of semi-conducting polarizable material of a thickness considerably less than one millimeter to a gradually increasing voltage, rendering a layer of said sheet polarized and able to withstand a voltage that is sufficient 35 to break down an unpolarized sheet layer of the same thickness.

In testimony whereof, I have signed my name to this specification this 20th day of February, 1926.

40

ABRAHAM JOFFÉ.

45

50

55

60

65